

## UNITED STATES PATENT OFFICE.

MONROE S. CLAWSON, OF UPPER MONTCLAIR, NEW JERSEY.

## NONRUSTING ALLOY.

No Drawing.

Application filed February 27, 1924. Serial No. 695,583.

To all whom it may concern:

Be it known that I, MONROE S. CLAWSON, a citizen of the United States, residing at Upper Montclair, in the county of Essex and

5 State of New Jersey, have invented certain new and useful Improvements in Nonrusting Alloys, of which the following is a specification.

This invention relates to alloys and has 10 for its object the formation of a non-rusting alloy suitable for making table ware, knife handles, building hardware, etc., the alloy having a somewhat silvery appearance making it attractive and ornamental in addition 15 to possessing sufficient hardness and toughness to insure proper durability.

An important object is the provision of 20 an alloy of this character which uses nickel as its base, there being also a high carbon content which, together with chromium and iron, will produce the hardness.

In carrying out the invention I make use 25 of the following ingredients used in substantially the proportions specified:

|           | Per cent. |
|-----------|-----------|
| Nickel    | 82 to 96  |
| Silicon   | 3 to 10   |
| Manganese | 1 to 5    |
| Copper    | ½ to 4    |
| Chromium  | 1 to 5    |
| Carbon    | .85 to 3½ |
| Iron      | 1 to 10   |

Quite naturally it may be necessary to use 30 certain reducing, deoxidizing and denitrogenizing elements such as titanium, alumi-

num, uranium, cerium and the like, which may be added to the above specified ingredients in various proportions, though naturally small amounts, to meet various conditions which may arise.

The above described alloy is really a nickel silicon combination with a high carbon content and owing to the presence of the other elements which combine well with a high percentage of carbon, I have found that the proportion of this particular element will not need to be disturbed or, as it is commonly called, "knocked down." The compound lends itself well to the making of table cutlery or so-called silver ware and innumerable other articles and it is particularly useful on account of its non-rusting qualities.

Having thus described my invention, what I claim as new and desire to secure by Letters Patent, is:

1. A non-rusting alloy consisting of nickel 60 82 to 96 percent, silicon 3 to 10 percent, manganese 1 to 5 percent, chromium 1 to 5 percent, carbon .85 to 3½ percent, iron 1 to 6 percent, and copper ½ to 4 percent, together with a small proportion of reducing, deoxidizing and denitrogenizing elements.

2. A non-rusting alloy consisting of nickel 65 82 to 96 percent, silicon 3 to 10 percent, manganese 1 to 5 percent, chromium 1 to 5 percent, carbon .85 to 3½ percent, iron 1 to 6 percent, and copper ½ to 4 percent, together with a trace of titanium or aluminum.

In testimony whereof I hereto affix my 70 signature.

MONROE S. CLAWSON.